# EUROPEAN PATENT SPECIFICATION

(11) **EP 1 878 026 B1**
(45) Date of publication and mention of the grant of the patent: **30.07.2008**
(21) Application number: 06732999.5
(22) Date of filing: 12.04.2006
(51) Int. Cl.: H01B 3/00, H01B 7/282

(54) **CABLE TAPE WITH OPEN-TEXTURE FIBROUS WEB**
KABELBAND MIT EINEM FASRIGEN GEWEBE OFFENER TEXTUR
BANDE POUR CABLE AVEC TISSU FIBREUX A TEXTURE OUVERTE

(30) Priority: 13.04.2005 EP 05075899
(43) Date of publication of application: 16.01.2008
(73) Proprietor: Lantor B.V., 3901 RG Veenendaal (NL)
(72) Inventor: KOHN, Frederik, Emiel, NL-3905 VS Veenendaal (NL)
(74) Representative: Hatzmann, Martin
(86) International application number: PCT/NL2006/000192
(87) International publication number: WO 2006/110033

(56) References cited:
- US-A1- 2003 041 473
- US-A1- 2004 229 536

## Description

The invention relates to a cable tape that can swell in a predetermined direction, as well as to a method for manufacturing such a cable tape and cables in which such cable tape is incorporated.

When manufacturing cables, for instance telecommunication cables, industrial (flexible) cables or energy cables (medium, high and ultra high voltage), a cable tape is often provided between the core or vein and the sheath, together, or not, with one or more other layers, for instance the copper wire screen in an energy cable. The function of this tape is often twofold, on the one hand to provide longitudinal watertightness and on the other hand to fill up empty spaces in the cable, so that this tape can serve as a cushioning for an overlying or an underlying layer, such as the copper wire screen in an energy cable. The tape can also serve as a bedding to provide protection against mechanical forces arising from pressure by metal parts such as the copper wire screen in an energy cable.

The longitudinal watertightness is obtained by incorporating a water-swelling material, typically a water-swelling powder, into the tape, while the filling properties are often obtained with a thick tape, obtainable, *inter alia,* by providing a foam or foamy structure, which is favourable with respect to providing a cushioning. A robust thick tape can be used for providing bedding properties.

The current types of cable tape for these applications are often manufactured by uniting two layers of basic web, a layer of swelling powder being provided between the two layers of basic web.

From EP-A-0 643 398 a cable tape is known, based on at least one fibrous web with water-swelling powder as swelling material. If the water-swelling powder is not enclosed by the first fibrous web and a second fibrous web, however, the swelling material can suffer from dusting in handling. On the other hand, if the fibrous web is applied on both sides, an incomplete filling of void volume in the cable may result upon water penetration, in particular in cases where the cable comprises a multitude of thick wires. In such cases the web on the inner side of the cable tape is not able to fit sufficiently well into the voids between the wires and thus prevents the swelling material from filling up these voids.

Also a so-called 'free swell' cable tape is known in the art from EP-A-0 540 815. This cable tape has a fibrous web on one side and water-swelling powder glued to it by e.g. a PVA-type polymer. In order to prevent dusting a second thin glue film is applied over the water-swelling powder, in a specific pattern. The thin glue film is water soluble so that it does not prevent the water-swelling powder from filling all void volume between the wires of the cable when contacted with water. However, the polymeric glue film may nevertheless interfere with the swelling capacity and swelling rate of the cable tape.

EP-A-0 378 940 describes a composite material comprising a mix of hydro-expandable powder and heat sealing powder, wherein these powders are in a sandwich construction between two solid supports of which at least one is at least partially water soluble. The heat sealing powder may however interfere with the swelling capacity and swelling rate of the composite material.

US-A-2003/0041473 describes a cable tape based on a fibrous web in which at least 0.5 wt.%, calculated on the weight of the cable tape, of non-expanded, pre-expanded, or expanded thermoplastic microspheres are incorporated. The fibrous web is not impregnated with binding agent.

US-A-2004/0229536 describes a water blocking tape for use in cable designs. The tape includes layers of non-woven fabric with one or more swellable water blocking compounds. The applied web does not have an open texture.

Accordingly, it is one of the objects of the invention to provide a cable tape which can swell in one direction, wherein the water-swelling powder is fixed without using glue, but while still preventing dusting. Also the tapes should be obtainable by a process using common, preferably existing apparatuses. With respect to the properties of the swelling tape, especially the swelling rate in the first minute is of importance, because it is most preferable that the longitudinal water transport is blocked quickly.

It is another object of the invention to provide a cable tape comprising water-swelling powder, which powder is able to effectively fill the void volume between different wires in the cable, in particular when the wires in the cable are large, e.g. having a diameter of 0.9 mm or more.

The inventors surprisingly found that these objects can be achieved by preparing a cable tape comprising water-swelling material in or on a fibrous base web, being covered by an open-textured fibrous web, wherein at least said fibrous base web, and optionally said open-textured fibrous web, is impregnated with at least one binding agent.

Figure 1 shows schematically a cross-section of a cable provided with a prior art cable tape. Figure 2 is a schematic representation of the cross-section of the same cable but now provided with the cable tape of the present invention.

When applying the cable tape of the present invention, upon water contact, the water-swelling material starts to swell and will penetrate through the open-textured fibrous web. Because the swollen powder extends beyond the open-textured fibrous web, an effective filling of the void volume between different wires in the cable is achieved. The open-textured fibrous web does not or negligibly inhibit the swelling capacity and swelling rate of the water-swelling powder. Furthermore, also dusting is efficiently prevented by providing the open-textured fibrous web on top of the water-swelling material.

The improved properties of the cable tape of the present invention are schematically illustrated in Figure 2, with reference to Figure 1, which represents the prior art. The cable of Figures 1 and 2 comprises a core (1) with adjacent wires (2). The cable is covered by outer sheath (3). In Figure 1, the prior art cable tape (4) is depicted in a swollen state, *viz.* after contacting water and being allowed to fully swell. As can be seen in Figure 1, the swollen tape is not able to cover the room between the wires (2) sufficiently, and thus voids (5) are left open, which allow for water transport in longitudinal direction, which is not desirable. The cable tape (4) in Figure 2 on the other hand, swells in such a manner that the swelling material can penetrate through the open-textured web (6), thereby filling the space between the wires (2) and thus a good blocking is obtained, since water is stopped from penetrating the cable any further.

Optionally, the invention also comprises expandable thermoplastic microspheres. It has been found that a combination of water-swelling powder and microspheres in the base web considerably increases the swelling properties of the web in water, in particular its swelling rate.

The invention also relates to a process for manufacturing the cable tape. The process of the present invention comprises the steps of providing a base web that is provided with a binding agent in or on the web and a water-swelling material in or on said web; applying a sealable open-textured fibrous web, which optionally may be provided with the same or a different binder, upon said base web; and effecting binding conditions to the resulting structure.

Preferably the binder that is applied in the base web is a heat sealable binder. More preferably, in case the open-textured web also comprises a binder, this binder is also a heat sealable binder. If a heat sealable binder is used, then the step of effecting binding conditions will normally comprise applying heat to the laminate structure.

The binding agent is typically applied to the base web or the open-textured fibrous web by contacting these webs with a solution or dispersion of these binders, e.g. by spraying, submerging, or foam bonding. In a preferred embodiment, the manufacturing comprises an additional incorporation and/or addition of non-expanded thermoplastic microspheres in and/or on the web support. This may be done at any moment prior to the drying, or prior to the drying and curing of the binding agent, and, during or after drying, or during or after drying and curing of the binding agent, an expansion of the microspheres.

The cable tape according to the invention, in its simplest form, is built up from three components. The fibrous base web, which is the starting point, can be a standard non-woven base web, originating from e.g. a carding machine or a spunbond machine for manufacturing non-woven webs. A woven can also be used.

The fibres of the base web are selected from natural fibres, synthetic fibres or a combination thereof. More in particular, polyester fibres, polypropene fibres, acrylic fibres, glass fibres, carbon fibres, polyamide fibres, aramid fibres and mixtures of two or more of these type of fibres are used. The weight of the base web can vary within broad limits, depending on the application. Current weights are from 10 g/m² to 250 g/m², preferably to 100 g/m². During manufacture, the web is bound with a binding agent, which, after drying or after drying and curing, gives the structure to the tape. Current binding agents are polyacrylates, styrene-butadiene rubbers, vinyl acetate, homo and copolymers and polyvinyl alcohol.

The fibrous webs can be both conducting as well as insulating. Conducting fibrous webs can be prepared by impregnating the fibrous webs with conductive carbon black. Conductivity and optionally shielding can also be obtained by using conductive fibres, for instance in the form of a blend of non-conductive fibres and conductive fibres, optionally in combination with a water-swelling material, or by an assembly of a conductive and a non-conductive fibre cloth which have been bonded onto each other. The conductive fibres can be e.g. metal fibres or metallised fibres.

The water-swelling material can be e.g. a powder, a paste, a gel, or the like. Water-swelling powder, also called "super-absorber", is a material which is commonly used in cable tape. Suitable swelling powders include polyacrylic acid swelling powders. Particularly suitable is slightly cross-linked, partially neutralised polyacrylic acid. It is preferably scattered on top of the fibrous base web. The binder on the surface will serve as an adhesive medium. It has appeared that swelling powder in and/or on the base web, together with microspheres in the base web, gives considerably better swelling properties, in particular a higher swelling rate, to the web, than when there are no microspheres in the web. The amount of water-swelling powder is preferably between 5 and 70 % by weight, calculated on the weight of the cable tape.

The open-textured fibrous web may in principle be made from the same material as the fibrous base web. An open-textured fibrous web in this context refers to a fibrous web which, when applied on top of a water-swelling powder, does not or negligibly inhibit the swelling capacity and swelling rate of said water-swelling powder, while preventing said water-swelling powder from dusting. In particular, the porosity of the open-textured fibrous web, measured as air permeability according to DIN 53887 at 2 mbar, is at least 5000 dm³/(s·m²). For providing a favourable swelling capacity and/or swelling rate, the porosity is preferably at least 7000 ls⁻¹m⁻² and most preferably at least 7500 ls⁻¹m⁻².

In particular in order to prevent dusting, the porosity is preferably 10000 ℓS⁻¹m⁻² or less, more preferably 9000 ℓs⁻¹m⁻² or less, most preferably 8500 ℓs⁻¹m⁻² or less.

As indicated above the open-textured fibrous web may be provided with a binding agent. This contributes to the sealability of the web. It is also possible that the web is "self-binding", e.g. it may be made from a material that is tacky or can be made tacky, e.g. under pressure or elevated temperature.

A very suitable material for use as open-textured fibrous web is a spunbond material.

The optional expandable thermoplastic microspheres comprises a thermoplastic skin, containing a gas. These microspheres are obtained by heating non-expandable spheres, provided with a blowing agent, to the correct temperature whereupon they expand. Such microspheres are, inter alia, commercially available under the name Expancel^{™} of Akzo Nobel. The thermoplastic polymer of which the cover consists can be based on methyl methacrylate and acrylonitrile, or on methyl methacrylate, acrylonitrile and vinylidene chloride. As a blowing agent, an organic material, such as an aliphatic hydrocarbon gas, for instance isobutane, pentane, or iso-octane, is provided in the microspheres. The diameter and the amount of microspheres together with the thickness determine to a large extent the filling properties (bedding properties) of the tape. Before swelling, the tape has a thickness of preferably 0.2 to 5 mm, more in particular 0.25 to 3 mm. The amount of microspheres is preferably between 5 and 20 % by weight, most preferably between 10 and 20 % by weight.

The web may also comprise other auxiliary substances, such as conductive materials (for instance metal particles), shielding or low-conductive materials (for instance carbon black). In particular for the manufacture of conductive, shielding or low-conductive tapes, it is desired to incorporate this sort of components. This effect can also be obtained by providing conductive fibres in the web in a suitable manner.

Without being limited to these dimensions, in an embodiment a cable tape according to the invention has a typical thickness of 0.2 to 2 mm before swelling, preferably 0.25 to 1.5 mm, and a typical width of 2 to 4000 mm, preferably 10 to 1000 mm.

The invention also relates to a cable, more in particular a telecommunication cable, industrial (flexible) cable and energy cable (medium high and ultra high voltage), manufactured using the cable tape according to the invention.

An important property of the cable tapes of the present invention is their blocking behaviour, in particular the resulting swelling speed (typically expressed as the increase in thickness in the first minute of swelling) and the resulting swell capacity (typically the thickness after becoming at equilibrium with an excess amount of water, which occurs e.g. after 10 minutes). An other parameter that is commonly used in this respect is the water penetration distance, which is the length of a cable that can be penetrated by water when water is applied at a constant pressure (e.g. of 1.1 bar) to an open end of the cable. The shorter the water penetration distance the better.

The water penetration distance can be measured by simulating the cable with glass tube (1) and a copper bar (2), shown in Figure 3. The bar has 20 grooves (3) along the long axis of the bar, which grooves are 2 mm deep and 2 mm wide. The cable tape is folded longitudinally around the bar with a 13.6 % overlap and the taped bar is surrounded by the glass tube in such a way that the smallest distance between the bar and the glass is at least 1 mm. The gap between the copper bar and the glass tube is connected to a water reservoir with a constant pressure of a 1 m high water column. The water penetration distance is the distance that the water penetrates into the gap between the copper bar and the glass tube until it is blocked by the cable tape. With cable tape according to the present invention water penetration distances of less than 1 m are easily obtained, using the above-mentioned measurement. Water penetration distances as low as 50 cm or less can also be obtained. When ordinary sandwich tape is used, the water penetration distance is more than 1.5 m (the length of the copper bar) within one minute.

### Example 1

A non-woven base fabric was produced by binding a carded web consisting of 22 gm⁻² polyester staple fibres with 13 gm⁻² heat sealable polyacrylate binder. A 10 gm⁻² open-textured spunbonded fibrous web, with a porosity measured as air permeability of 6700 ls⁻¹m⁻², consisting of polyamide-6,6 filaments was impregnated with 2-5 gm⁻² of the same binder. The cable tape was produced thereof by scattering 40 gm⁻² swelling powder on top of the non-woven base web, and subsequently covering the underlayer plus swelling powder with the impregnated open-textured fibrous web. Thereafter an effective bonding between the two layers enclosing the swelling powder was obtained by applying heat and pressure in a calendering process. A swelling height of 22 mm and a swelling speed of 20 mm in the first minute was measured. In the water penetration test as described above a water penetration distance of 40 cm was measured.

## Claims

1. A cable tape comprising water-swelling material in or on a fibrous base web, being covered by an open-textured fibrous web, wherein at least said fibrous base web, and optionally said open-textured fibrous web, is impregnated with at least one binding agent.

2. Cable tape according to claim 1, wherein said binding agent is a heat sealable binding agent.

3. Cable tape according to any of the previous claims, wherein said open-textured fibrous web has a porosity measured as air permeability of at least 5000 ls⁻¹m⁻², preferably 5000-10000 ls⁻¹m⁻², more preferably of 7000-9000 ls⁻¹m⁻², and most preferably of 7500 - 8500 ls⁻¹m⁻².

4. A cable tape according to any of the previous claims, wherein said cable tape further comprises non-expanded, pre-expanded or expanded thermoplastic microspheres.

5. A cable tape according to any of the previous claims, wherein the amount of water-swelling material is between 5 and 70 % by weight, calculated on the weight of the cable tape.

6. A cable tape according to any of the preceding claims, which has a thickness before swelling of 0.2 to 5 mm, preferably 0.25 to 3 mm.

7. A cable tape according to any of the preceding claims, which has a width of 2 to 4000 mm, preferably 10 to 1000 mm.

8. A cable tape according to any of the claims 2-7, wherein the amount of said thermoplastic microspheres is between 1 and 20 % by weight, preferably between 5 and 20 % by weight, calculated on the weight of the cable tape.

9. A cable tape according to claims 2-8, wherein the average diameter of the not yet expanded thermoplastic microspheres is between 10 and 100 µm.

10. A cable tape according to any of the previous claims, wherein the fibres of said fibrous base web are selected from the group consisting of natural and synthetic fibres, more in particular polyester fibres, polypropylene fibres, acrylic fibres, glass fibres, carbon fibres, polyamide fibres, and mixtures of two or more of these types of fibres.

11. A cable tape according to any of the previous claims, wherein the fibres of said open-textured fibrous web are selected from the group consisting of natural and synthetic fibres, more in particular polyester fibres, polypropylene fibres, acrylic fibres, glass fibres, carbon fibres, polyamide fibres, and mixtures of two or more of these types of fibres.

12. A cable tape according to any of the preceding claims, wherein the web has cushioning properties and/or bedding properties.

13. A cable tape according to any of the preceding claims, which is electrically conductive.

14. A cable tape according to any of the preceding claims, wherein the tape is suitable for use in telecommunication cable, industrial (flexible) cable and/or energy cable (medium, high and ultrahigh voltage).

15. A cable comprising a cable tape according to any of the previous claims, preferably having a water penetration distances of less than 1 m, more preferably 50 cm or less.

16. A method for manufacturing a cable tape according to any of the preceding claims comprising manufacturing a base web, providing a binding agent in the web, and binding the web by drying and curing the binding agent, while the water-swelling material, at any moment prior to, during, or after the drying, or prior to, during, or after the drying and curing of the binding agent, is incorporated in and/or added on the base web, and applying a sealable open-textured fibrous web on top of the water-swelling material.

17. A method according to claim 16, further comprising the incorporation and/or addition of non-expanded thermoplastic microspheres at any moment prior to the drying, or prior to the drying and curing of the binding agent, in and/or on the base web, and, during or after drying, or during or after drying and curing of the binding agent, expanding of the microspheres.

## Patentansprüche

1. Kabelband mit einem wasserquellfähigen Material in oder auf einer Faserbasisbahn, die durch eine Faserbahn mit offener Textur bedeckt ist, wobei wenigstens die Faserbasisbahn, und optional die Faserbahn mit offener Textur, mit wenigstens einem Bindemittel imprägniert ist.

2. Kabelband nach Anspruch 1, wobei das Bindemittel ein heißsiegelbares Bindemittel ist.

3. Kabelband nach einem der vorhergehenden Ansprüche, wobei die Faserbahn mit offener Textur eine Porosität messen als Luftdurchlässigkeit von wenigstens 5000 ls⁻¹m⁻², vorzugsweise 5000 - 10.000 ls⁻¹m⁻², bevorzugter von 7000 - 9000 ls⁻¹m⁻² und besonders bevorzugt von 7500 - 8500 ls⁻¹m⁻², hat.

4. Kabelband nach einem der vorhergehenden Ansprüche, wobei das Kabelband weiter nicht expandierte, vorexpandierte oder expandierte thermoplastische Mikrokügelchen aufweist.

5. Kabelband nach einem der vorhergehenden Ansprüche, wobei die Menge des wasserquellfähigen Materials 5 bis 70 Gew.% berechnet auf Grundlage des Gewichts des Kabelbandes beträgt.

6. Kabelband nach einem der vorhergehenden Ansprüche, das vor dem Quellen eine Dicke 0,2 bis 5 mm, vorzugsweise von 0,25 bis 3 mm, hat.

7. Kabelband nach einem der vorhergehenden Ansprüche, das eine Breite von 2 bis 4000 mm, vorzugsweise von 10 bis 1000 mm, hat.

8. Kabelband nach einem der Ansprüche 2 - 7, wobei der Anteil der thermoplastischen Mikrokügelchen berechnet auf Grundlage des Gewichts des Kabelbandes zwischen 1 und 20 Gew.% liegt, vorzugsweise zwischen 5 und 20 Gew.%.

9. Kabelband nach einem der Ansprüche 2 - 8, wobei der mittlere Durchmesser der noch nicht expandierten thermoplastischen Mirkokügelchen zwischen 10 und 100 µm beträgt.

10. Kabelband nach einem der vorhergehenden Ansprüche, wobei die Fasern der Faserbasisbahn ausgewählt sind aus der Gruppe bestehend aus natürlichen und synthetischen Fasern, insbesondere Polyesterfasern, Polypropylenfasern, Acrylfasern, Glasfasern, Kohlenstofffasern, Polyamidfasern und Gemische aus zwei oder mehr dieser Arten von Fasern.

11. Kabelband nach einem der vorhergehenden Ansprüche, wobei die Fasern der Faserbahn mit offener Textur ausgewählt sind aus der Gruppe bestehend aus natürlichen und synthetischen Fasern, insbesondere Polyesterfasern, Polypropylenfasern, Acrylfasern, Glasfasern, Kohlenstofffasern, Polyamidfasern und Gemische aus zwei oder mehr dieser Arten von Fasern.

12. Kabelband nach einem der vorhergehenden Ansprüche, wobei die Bahn Kisseneigenschaften und/oder Polstereigenschaften hat.

13. Kabelband nach einem der vorhergehenden Ansprüche, das elektrisch leitfähig ist.

14. Kabelband nach einem der vorhergehenden Ansprüche, wobei das Band zur Verwendung in einem Telekommunikationskabel, in einem industriellen (flexiblen) Kabel und/oder einem Energiekabel (mittlere Spannung, Hochspannung oder Ultrahochspannung) geeignet ist.

15. Kabel mit einem Kabelband nach einem der vorhergehenden Ansprüche, vorzugsweise mit einer Wassereindringdistanz von weniger als 1 m, bevorzugter von 50 cm oder weniger.

16. Verfahren zum Herstellen eines Kabelbandes nach einem der vorhergehenden Ansprüche, bei dem ein Basisband hergestellt, ein Bindemittel in dem Band bereitgestellt wird und die Bahn abbinden gelassen wird, indem das Bindemittel getrocknet und ausgehärtet wird, während das wasserquellfähige Material zu irgendeinem Zeitpunkt vor, während oder nach dem Trocknen oder vor, während oder nach dem Trocknen und Aushärten des Bindemittels in die Basisbahn eingebracht oder darauf hinzugefügt wird und eine siegelbare Faserbahn mit offener Textur oben auf das wasserquellfähige Material aufgebracht wird.

17. Verfahren nach Anspruch 16, bei dem weiter nicht expandierte thermoplastische Mikrokügelchen in und/oder auf die Basisbahn eingebracht oder hinzugefügt werden zu irgendeinem Zeitpunkt vor dem Trocknen oder vor dem Trocknen und Aushärten des Bindemittels, und bei dem während oder nach dem Trocknen oder während und nach dem Trocknen und Aushärten des Bindemittels die Mikrokügelchen expandiert werden.

## Revendications

1. Bande pour câble comprenant un matériau gonflant à l'eau situé dans ou sur un tissu de base fibreux, lequel est recouvert d'un tissu fibreux à texture ouverte, dans laquelle au moins ledit tissu de base fibreux, et éventuellement ledit tissu fibreux à texture ouverte, est imprégné d'au moins un liant.

2. Bande pour câble selon la revendication 1, dans laquelle ledit liant est un liant thermoadhésif.

3. Bande pour câble selon l'une quelconque des revendications précédentes, dans laquelle ledit tissu fibreux à texture ouverte présente une porosité mesurée en termes de perméabilité à l'air d'au moins 5000 ls⁻¹m⁻², de préférence de 5000 à 10000 ls⁻¹ m⁻², et de préférence encore de 7000 à 9000 ls⁻¹m⁻², et idéalement de 7500 à 8500 ls⁻¹m⁻².

4. Bande pour câble selon l'une quelconque des revendications précédentes, dans laquelle ladite bande pour câble comprend en outre des microsphères thermoplastiques non expansées, pré-expansées ou expansées.

5. Bande pour câble selon l'une quelconque des revendications précédentes, dans laquelle la quantité de matériau gonflant à l'eau est comprise entre 5 et 70 % en poids, rapporté au poids de la bande pour câble.

6. Bande pour câble selon l'une quelconque des revendications précédentes, dont l'épaisseur avant gonflement est comprise entre 0,2 et 5 mm, de préférence entre 0,25 et 3 mm.

7. Bande pour câble selon l'une quelconque des revendications précédentes, dont la largeur est de 2 à 4000 mm, de préférence de 10 à 1000 mm.

8. Bande pour câble selon l'une quelconque des revendications 2 à 7, dans laquelle la quantité desdites microsphères thermoplastiques est comprise entre 1 et 20 % en poids, de préférence entre 5 et 20 % en poids, rapporté au poids de la bande pour câble.

9. Bande pour câble selon les revendications 2 à 8, dans laquelle le diamètre moyen des microsphères thermoplastiques non encore expansées est compris entre 10 et 100 µm.

10. Bande pour câble selon l'une quelconque des revendications précédentes, dans laquelle les fibres dudit tissu de base fibreux sont choisies dans le groupe formé par les fibres naturelles et synthétiques, plus particulièrement les fibres de polyester, les fibres de polypropylène, les fibres acryliques, les fibres de verre, les fibres de carbone, les fibres de polyamide et les mélanges de deux de ces types de fibres ou plus.

11. Bande pour câble selon l'une quelconque des revendications précédentes, dans laquelle les fibres dudit tissu fibreux à texture ouverte sont choisies dans le groupe formé par les fibres naturelles et synthétiques, plus particulièrement les fibres de polyester, les fibres de polypropylène, les fibres acryliques, les fibres de verre, les fibres de carbone, les fibres de polyamide et les mélanges de deux de ces types de fibres ou plus.

12. Bande pour câble selon l'une quelconque des revendications précédentes, dans laquelle le tissu a des propriétés d'amortissement et/ou de calage.

13. Bande pour câble selon l'une quelconque des revendications précédentes, qui est conductrice d'électricité.

14. Bande pour câble selon l'une quelconque des revendications précédentes, dans laquelle la bande convient à une utilisation dans un câble de télécommunications, un câble industriel (flexible) et/ou un câble électrique (moyenne, haute et très haute tension).

15. Bande pour câble selon l'une quelconque des revendications précédentes, présentant de préférence une distance de pénétration d'eau inférieure à 1 m, de préférence de 50 cm ou moins.

16. Procédé de fabrication d'une bande pour câble selon l'une quelconque des revendications précédentes, consistant à fabriquer un tissu de base, à prévoir un liant dans le tissu et à lier le tissu en faisant sécher et durcir le liant, tandis que le matériau gonflant à l'eau est incorporé dans et/ou ajouté sur le tissu de base à n'importe quel moment avant, pendant ou après le séchage ou avant, pendant ou après le séchage et durcissement du liant, et à appliquer par-dessus le matériau gonflant à l'eau un tissu fibreux adhésif à texture ouverte.

17. Procédé selon la revendication 16, consistant en outre à incorporer et/ou ajouter des microsphères thermoplastiques non expansées dans et/ou sur le tissu de base à n'importe quel moment avant le séchage ou avant le séchage et durcissement du liant et à réaliser l'expansion des microsphères pendant ou après le séchage ou pendant ou après le séchage et durcissement du liant.
